

## UNITED STATES PATENT OFFICE

2,052,714

ALLOY AND METHOD OF MAKING  
THE SAMEFriedrich Kempka, New York, N. Y., assignor of  
one-half to Edward Van Hoofstadt, North Val-  
ley Stream, Long Island, N. Y.No Drawing. Application April 10, 1934,  
Serial No. 719,852

2 Claims. (Cl. 148-2)

This invention relates primarily to an alloy of cast iron and a metal derived from or containing iron, and especially useful in patching or repairing other metals derived from or containing iron.

5 One object of the invention is to provide an alloy which may be worked conveniently at relatively low temperatures and may be applied to worn or broken parts in such manner as to form an economical repair, so constituted that the 10 repair thus provided is more durable than the original material and can be accomplished for a relatively small fraction of the cost of a replacement part.

One practical illustration of the method of 15 forming the alloy of this invention is as follows. As a first step, apply sufficient temperature to say, one pound of cast iron, in the presence of one ounce of borax, to cause the cast iron to flow sufficiently to bring about a fusing together of the borax and cast iron. The iron used in gray 20 iron castings works very well for this purpose. The temperature applied should be sufficient to cause this fusing, but should be maintained as low as possible while still bringing about this result. I have obtained very satisfactory results 25 through the use of an acetylene flame applied to the iron and borax in such manner that, as the heat melts the iron and fuses it with the borax, the fused mass drops out of the zone of the 30 flame, so that there is not a too prolonged or excessive heating. The fused mass is permitted to drop into water and forms globules or drops of different sizes, although, in practice, the heating may be carried on in an electric or other furnace, so controlled as to cause the fusing referred to without excessive heating and the fused 35 material may be removed in a crucible or otherwise, and thereafter poured into water. The purpose of dropping the fused material into 40 water is primarily to eliminate impurities from the material and this may be accomplished in any other equivalent way known to the art if desired.

The globules or drops obtained when dropped 45 into water may be in different sizes or may be reheated and cast in appropriate molds, if preferred, but it is thoroughly satisfactory and convenient to leave them in the condition in which they are initially formed for further use. They 50 constitute the basis of the alloy of this invention, and are the product of the first step of the process.

As a second step in the process, I fuse together 55 in substantially the same manner as in the first step the materials which are to be alloyed with the product of the first step. These materials may vary without departing from the invention, but they embody in every instance a metal derived from or containing iron. A wide variety 60 of such metals may be employed, such, for ex-

ample, as mild steels, nickel steel, tool steel or practically any other steel or other alloy which may be considered best suited for the particular purpose for which the alloy is to be used. I have found, however, that very satisfactory results can be had by using a cheap mild steel in the interest of economy. Thus I may take, e. g., one-half pound of mild steel. This together with one-half ounce of borax and preferably one-quarter ounce of copper are fused together in the same 10 manner as the first step of the process and the molten material is permitted to fall in the form of drops or globules into the water as before to form the product of the second step of this process. 15

Having obtained separately and independently two distinct products from the first and second steps of the process, these two products are melted together with the addition of an appropriate flux, say, one ounce of borax in a crucible or in 20 any other suitable manner and to a temperature wherein they will thoroughly admix with one another. During this third step of the method, I preferably employ accompanying agitation of the mass in order to get a thorough admixture of the 25 constituents. This agitation may be obtained by a flame or mechanically, as may be desired, but in this third step of the method, as well as in the prior steps, the temperature must be kept as 30 low as possible, for if too high a temperature is used, the resulting end product becomes so hard that it cannot be worked and cannot be softened except by prolonged annealing.

After the constituents of the first and second steps are thoroughly admixed in the third step, 35 as stated, the resulting admixture is run out into suitable molds for the purpose of forming the end product of the process. The resulting alloy material is hard and brittle and can be shaped by tools only after heat treatment to soften the 40 same.

I have expressly referred to the employment of copper and have described a proportion of about 3 per cent, by weight, of the mild steel used, i. e., between 1 and 2 per cent of the entire mass. 45 This copper I prefer to employ because I find that it assists in making the resulting alloy free flowing and that the alloy works better with the copper therein. 3 per cent copper, as stated, gives an economical composition and a thoroughly sat- 50 isfactory one in practice. I may, however, use less or dispense with the copper entirely if a very hard brittle alloy is desired, or I may use slightly more copper than stated, but as the percentage of copper is increased, there is a decrease in the 55 hardness of the final product and if too much copper is added, the copper tends to separate during the welding operation and accumulate as a surface shell for the resulting weld. The copper therefore should be kept down to a point beyond 60

which this formation of a shell will not occur if a hard surface is desired in the final product.

The alloy of the present invention resulting from the novel steps hereinbefore enumerated may be used in various ways, but is particularly useful as a patching material. As such, it may be applied to worn or broken parts through the employment of an acetylene torch or any other suitable source of heat, following substantially the technique of the welding art with certain exceptions. That is to say, the material is used like ordinary welding rod and is applied in the same manner. It is built up to the desired extent over the part to be repaired or patched and at temperatures sufficient to produce a proper weld, but not so high as to overheat. In other words, the material should be heated no more than necessary to obtain a proper weld. After the alloy has been applied, as stated, the assembled parts should be permitted to slowly cool. The cooling should be relatively slow and should not be speeded up. It is preferably accomplished in the absence of drafts and if desired may be controlled by ovens or otherwise, so that return to room temperature is slowly brought about. When thus cooled, the alloy material added is relatively soft. It can be worked with tools, files, cutters, etc., and thus shaped and proportioned to the desired form and dimensions.

After these shaping and working operations, the substantially finished work is preferably subjected to heat, the added alloy portion being raised to a temperature of approximately cherry red and immediately quenched, preferably in water. My experience has shown that the higher the temperature the harder the product and thus the temperature during this step will be used as desired. During this last heating and quenching step, there is practically no deformation or distortion of the metal, so that if parts have been properly machined to shape and size, they will remain so through the last mentioned step. After hardening as stated, the material is so hard that it cannot be worked with file or tools although it may be polished with appropriate polishing materials if desired. Nevertheless it is of appreciably greater hardness than any of the separate materials which have entered into its manufacture and will withstand wear and vibration almost indefinitely. It is notable, however, that the material does not possess, in finished hardened form, any appreciable degree of ductility. It has a tendency to fracture if stretched above a relatively low elastic limit. It commends itself particularly for use in patching and like manufacturing or repair operations because of the economy of its manufacture and application and by reason of the remarkable hardness and resistance to wear of the finished job.

The alloy of the present invention does not possess any great degree of inherent tensile strength and is thus not intended primarily for use as a material for the manufacture of small parts. If the parts are relatively large and rugged, however, the alloy may be so used, but I have found in practice that where the material in my invention is backed up or used upon a foundation of some other metal, from which it can derive its inherent strength, it is highly satisfactory for many uses and particularly those where a high resistance to wear is of primary importance.

I have applied the alloy of this invention in the manner described not only to cast iron, but

to a wide variety of steels and irons and I have found that when applied to these other metals or alloys by welding operations, as hereinbefore stated, a very satisfactory bond is obtainable.

I have hereinbefore referred to the fact that after the alloy of this invention has been applied to another metal and allowed to cool slowly, that it can be readily worked with cutting tools, files, etc., for it is of a sufficient degree of softness to readily permit of efficient shaping in this way. For example, the alloy made up of cast iron, mild steel and copper in the proportions hereinbefore stated has been found, when in such relatively soft workable condition, to have, as shown by various tests, a Rockwell hardness (C scale) of between 35 and 45, whereas when hardened and in its final form for use as a wear resistant, it has been found to possess a Rockwell hardness of from 51 to 57. When it is borne in mind that the well known "Stellite" has a 57 Rockwell hardness, some indication may be had of the remarkable hardness of which the alloy of this invention is capable in its finished condition and this accounts largely for its great ability to withstand wear.

In the foregoing detailed description, I have set forth the preferred manner of practising the present invention. I have set forth the various steps of the process whereby the alloy is compounded. I have described the alloy and I have described a method whereby said alloy may be used to produce wear resisting parts of a high degree. The invention embodies the foregoing aspects severally, as well as collectively, and is to be understood as fully commensurate with the appended claims.

Having thus fully described the invention, what I claim as new and desire to secure by Letters Patent is:

1. The process which consists in the following steps, utilizing substantially the proportions stated; namely, fusing together one pound of cast iron and 1 ounce of borax to form one product, fusing together  $\frac{1}{2}$  pound of mild steel and  $\frac{1}{2}$  ounce of borax to produce a second product, then fusing together the first and second products with an additional 1 ounce of borax, and permitting the combined product to cool to room temperature, thereafter welding a quantity of this combined product to an independent metallic body in the presence of a borax flux to add to said body a mass of said combined product and allowing said mass to slowly cool to room temperature, thereafter machining the applied mass to the desired shape and size, thereafter heating said applied mass to a hardening temperature and thereupon quenching the said applied mass.

2. The herein described process which consists in fusing together cast iron and borax, separately fusing together mild steel and borax, then fusing together the resulting two products with the addition of further borax to provide a combined product, thereafter welding a quantity of the combined product to a separate metallic body to form a mass of said combined product thereon and allowing the same to slowly cool to room temperature, thereafter working the applied mass to the desired shape and dimension with appropriate tools, thereafter raising the temperature of the thus worked applied mass to a hardening temperature and thereupon quenching the same.

FRIEDRICH KEMPKA.